

## UNITED STATES PATENT OFFICE

ARCHIBALD H. Vining, of San Jose, California

## ADHESIVE

No Drawing.

Application filed January 30, 1930. Serial No. 424,725.

This invention relates particularly to an adhesive to be used for temporarily mounting a mask upon a surface which it is desired to protect while an exposed surface is being sprayed with paint or otherwise treated.

The objects of the invention are to provide an adhesive that may be spread evenly upon a masking paper or other suitable material without causing the same to warp; that will not squeeze out along the edge when the mask of which it forms a part is applied to the surface to be protected; that will not mix along the edge with the lacquer or other material being applied; that will permit arranging the coated material in layers so that a plurality of duplicate masks may be cut at the same time; that leaves a clean easily polished surface upon removal of the mask; that is efficient in all temperatures to which it is ordinarily subjected.

My composition consists, essentially, of a mixture of beeswax, lanolin, castor oil, and Venice turpentine, which may be thinned by the addition of spirits of turpentine.

In preparing the composition I prefer to use the ingredients in about the following proportions—viz., fifty-two per cent beeswax, twenty-four per cent lanolin, nine per cent castor oil, and fifteen per cent Venice turpentine, but these proportions may be varied to meet various conditions presented by temperature, grade of materials used, character of material to be coated, etc.

A beeswax is used for the body material because of its adhesive qualities, its uniform consistency, and its characteristic reaction to heat; the lanolin because it retards drying and causes the composition to resist combining with the lacquer, paint, varnish, etc., at the edge of the mask when in use; the castor oil because it counteracts the tendency of the Venice turpentine to dry out the composition, and the Venice turpentine because it mixes readily with the wax and provides the desired glue-like adhesiveness.

When this composition is used the mask may be readily removed from the surface to which it is applied, and when sheets coated with it are disposed in layers to permit cutting a number of duplicates, they may be

readily separated after cutting. Furthermore, when stencils are applied with this composition the ties may be cut out before the spraying or brush work is begun, obviating the necessity of finishing the work later after the stencil is removed. 55

The composition above described is prepared by mixing the ingredients while hot, and then spreading upon the paper. This composition will not squeeze out along the edge of the paper when it is applied to a surface, and when the paper is removed from the protected surface the said protected surface may be simply polished instead of being subjected to a cleaning such as is ordinarily required. 60 65

I claim:

- An adhesive composition for masks consisting of beeswax, lanolin, and a turpentine having the consistency of Venice turpentine. 70
- An adhesive composition for masks consisting of beeswax, lanolin, castor oil, and Venice turpentine. 75
- An adhesive composition for masks consisting of about fifty-two per cent beeswax, twenty-four per cent lanolin, nine per cent castor oil and fifteen per cent Venice turpentine.
- An adhesive composition for masks consisting of not less than 52% beeswax, not less than 24% lanolin, not less than 9% castor oil, and not less than 15% Venice turpentine. 80

ARCHIBALD H. Vining.

85

90

95

100